# EUROPEAN PATENT SPECIFICATION

(11) **EP 0 054 061 B1**
(45) Date of publication and mention of the grant of the patent: **03.10.1984**
(21) Application number: 81901923.3
(22) Date of filing: 22.06.1981
(51) Int. Cl.: B22C 9/00

(54) **A METHOD OF PRODUCING FROZEN CASTING MOULDS OR CORES**
VERFAHREN ZUR HERSTELLUNG GEFRORENER GIESSFORMEN ODER KERNE
PROCEDE DE PRODUCTION DE MOULES DE COULEE OU NOYAUX SOLIDIFIES

(30) Priority: 23.06.1980 DK 2675/80
(43) Date of publication of application: 23.06.1982
(73) Proprietor: DANSK INDUSTRI SYNDIKAT A/S, DK-2730 Herlev (DK)
(72) Inventor: JESPERSEN, Emil, DK-2600 Glostrup (DK); SINGH, Bakshi Brijindra, DK-2970 Horsholm (DE)
(74) Representative: Lehn, Werner, Dipl.-Ing.
(86) International application number: DK8100062
(87) International publication number: WO8200015

## Description

The invention relates to a method of producing frozen casting moulds or cores of a granular material and a binder in a mould chamber or a core box, comprising the use of a freezable binder which is in a gas or liquid state at positive temperatures calculated in °C.

The specification of US-A-4 150 704 teaches a method in which the mould sand is admixed with a controlled quantity of water which after moulding is frozen to ice in a certain depth from the surface that is caused to contact molten metal e.g. by placing a layer of so-called dry ice or spraying liquid nitrogen on the surface. This gives a very strong mould surface which retains its strength and shape until the surface of the metal has solidified. As the metal gives off its heat, the water melts and evaporates so that the mould begins collapsing without the use of mechanical means. Practically no smoke is developed in the casting process, and the mould sand can be reused right away.

An article in the Russian magazine Liteinoe Proizvodsto, 1975, no. 5, p. 21-22, describes the freezing of a sand mould containing 3 to 7% water by means of a coolant that circulates through the evaporator in a cooling system and through the mould.

Freezing of the added water is by nature a rather slow process, and consequently it takes a relatively long time from the moment when the moulding process is finished until the mould has frozen deep enough to be able to resist the effect of molten metal for a sufficiently long time, and this in turn causes the overall mould production to become considerably more time- consuming than the conventional mould manufacturing process.

In SU-A-428843 it has been proposed to shorten the process time by the application of a hollow pattern, to the cavity of which a cooling medium is continuously supplied. Another proposal set forth in PL-A-21861 1 is to freeze liquid in sand moulds or cores by precooling the pattern or core box in question which is to be engaged by the sand. PL-A-224193 describes the application of a disposable pattern of a permeable material which disintegrates when exposed to the molten metal and through which liquid gas is applied to the mould sand. Furthermore, it has in SU-A-718215 been proposed to mix the moulding sand with solidified carbon dioxide before applying the moulding sand on the pattern, said carbon dioxide serving to cool the moulding sand which contains about 4% water. DE-Al-29 09 839 discloses a mould forming process, in which two streams of sand lead to a mixing device. In one stream water is added to the sand, whereas the sand in the other stream is subjected to a cooling agent such as liquid nitrogen. From the mixing device the mixture of moistened and cooled sand is supplied to the mould box.

According to the present invention a still further reduction of the time needed for the production of frozen casting moulds or cores may be obtained by a method in which the binder has been frozen before it is mixed with granular material. Thereby the moulding time is substantially reduced to the time it takes to fill the flask or core box with the mixture of and and binder and to compress said mixture sufficiently around the pattern or adjacent the walls of the core box cavity to enable the binder to putty the sand corns together.

As stated in claim 2 a mould binder may be used which is present in the form of fine, dendritic particles, e.g. snow, in the mould material, and a compression during the moulding process may entail that the binder obtains part of or its entire binding capacity depending upon the temperature conditions at the time of the mould manufacturing process.

The mould binder used may, as stated in claim 3, also be present in the form of a finely divided powdered material, e.g. ice, in the mould material, and a compression during the moulding process may entail that the binder obtains part of or its entire binding capacity depending upon the temperature conditions at the time of the mould manufacturing process.

When a suitable mixture of granular material and snow or broken ice is compressed in a mould box, the snow or the ice may thus be caused to bind the grains of the material together to impart a cohesive force to the mould or the core sufficient for it to resist the effect from liquid metal which is poured down into the finished mould with or without cores. A corresponding effect can be achieved by injecting one of the mentioned mixtures of mould material into a core box with a sufficiently great force and at a sufficiently great rate.

The precooled binder in the form of pulverized material may, as stated in claim 4, also be combined with liquid gas. This permits the temperature of the mould material to be reduced to a very low value before and during the moulding process and during the immediately following casting process. The mixture must be homogeneous and easy flowing.

Actually, there is nothing to prevent the use of conventional setting binders. Thus, to form a binder there may be used water glass and liquid carbon dioxide, as stated in claim 5, or a mixture of polyisocyanate and phenol resin which is activated by precooled, liquid dimethylethyl amine or triethyl amine, as stated in claim 6. This provides for a reduction in the use of an environmentally harmful binder.

To obtain a better resistance to the heat effect of the molten metal and thereby a delay in the heating of the mould or the core in the casting process, the granular material used for the formation of the mould or the core may have been deep frozen in advance in a manner known per se. Also the process ingredients may have been deep-frozen in advance by means of an admixed freezing agent such as liquid gas. The use of an inert gas obviates any risk of chemical attacks on the equipment used for the process or for chemical reactions with the casting metal.

The required cooling may also in a manner known per se be effected or be supported by deep-freezing the parts of the apparatus which the mould material contacts during the moulding process. In the production of casting moulds, particularly the pattern board which contacts the same mould surface as the molten metal does later, may have been deep-frozen in advance, and a core box deep-frozen in advance may be used in the production of cores. Also, the core box with the core or cores may be cooled simultaneously and additionally, e.g. with liquid gas.

A specific embodiment of the method of the invention in the production of casting moulds comprises the use of deep-frozen disposable patterns of a material which evaporates when heated, as stated in claim 7, and this material may expediently have been deep-frozen and foamed, as stated in claim 8. Such patterns may be produced currently in a particular bifurcate pattern mould box corresponding to a conventional core box and be placed in a closed chamber, following which the space between the pattern and the walls of the chamber is filled with the moulding material which is cooled by the pattern and may additionally have been cooled in advance as mentioned above. After the moulding process is finished the pattern evaporates rapidly owing to the heat received. This obviates the inconvenient development of gas, which otherwise takes place in the moulding of disposable patterns. This embodiment of the method results in particularly accurate castings because the inaccuracies which in the conventional mould manfacturing process result from wear on the pattern board caused by shootings of sand, are avoided. Moreover, bifurcation of the mould box is not required when readily evaporable patterns are used.

As stated in the characterizing portion of claim 9, apparatus for the production of casting moulds and/or apparatus for the production of cores are used, the apparatus or parts of it being contained in a cooling chamber. The necessary temperature conditions may be readily and constantly maintained so that valuable production time is not lost in waiting for cooling.

## Claims

1. A method of producing frozen casting moulds or cores of a granular material and a binder in a mould chamber or a core box, comprising the use of a binder which is in a gas or liquid state at positive temperatures calculated in °C, characterized in that the binder has been frozen before it is mixed with the granular material.

2. A method according to claim 1, characterized in that a mould binder is used which is present in the form of fine, dendritic particles e.g. snow, in the mould material, and that compression during the moulding process causes the binder to obtain part of or its entire binding capacity depending upon the temperature conditions at the time of the mould manufacturing process.

3. A method according to claim 1, characterized in that a mould binder is used which is present in the form of finely divided powdered material, e.g. ice, in the mould material, and that compression during the moulding process causes the binder to obtain part of or its entire binding capacity depending upon the temperature conditions at the time of the mould manufacturing process.

4. A method according to claim 3, characterized in that the precooled binder in the form of pulverized material is combined with liquid gas.

5. A method according to claim 1, characterized by the use of water glass and liquid carbon dioxide to form a binder.

6. A method according to claim 1, characterized in that a mixture of polyisocyanate and phenol resin which is activated by pre-frozen, liquid dimethylethyl amine or triethyl amine, is used for the formation of a binder.

7. A method according to any of the claims 1-6 in the production of casting moulds, characterized by the use of deep-frozen disposable patterns of a material which evaporates when heated.

8. A method according to claim 7, characterized by the use of disposable patterns manufactured from a deep-frozen, foamed material.

9. A method according to any one of the preceding claims, characterized by the use of apparatus for the production of casting moulds and/or apparatus for the production of cores, the apparatus or parts of it being contained in a cooling chamber.

## Revendications

1. Procédé de production de moules de coulée ou de noyaux d'un matériau granulaire et d'un liant dans une chambre de moulage ou une boîte à noyau, comprenant l'utilisation d'un liant qui est dans un état gazeux ou liquide à une température positive calculée en °C, caractérisé en ce que le liant a été gelé avant qu'il soit mélangé avec le matériau granulaire.

2. Procédé selon la revendication 1, caractérisé en ce qu'un liant de moulage est utilisé, qui se présente sous forme de particules fines, dendritiques, par exemple de la neige, dans le matériau de moulage, et en ce que la compression pendant le processus de moulage a pour effet que le liant acquiert une partie ou la totalité de sa capacité de liaison en fonction des conditions de température au moment du processus de production du moule.

3. Procédé selon la revendication 1, caractérisé en ce qu'un liant de moulage est utilisé, qui se présente sous forme d'une substance poudreuse finement divisée, par exemple de la glace, dans le matériau de moulage, et en ce que la compression pendant le processus de moulage a pour effet que le liant acquiert une partie ou la totalité de sa capacité de liaison en fonction des conditions de température au moment du processus de production du moule.

4. Procédé selon la revendication 3, caractérisé en ce que le liant préalablement refroidi et sous forme d'une substance pulvérisée est combiné avec du gaz liquide.

5. Procédé selon la revendication 1, caractérisé par l'usage de verre soluble et du dioxyde de carbone liquide pour former un liant.

6. Procédé selon la revendication 1, caractérisé en ce qu'on utilise, pour la formation d'un liant, un mélange de polyisocyanate et de résine de phénol, qui est activé par du diméthyléthyl amine ou du triéthyl amine liquide, congelé préalablement.

7. Procédé selon l'une des revendications 1 à 6 pour la production de moules de coulée, caractérisé par l'utilisation de modèles perdus surgelés d'une substance qui s'évapore lorsqu'elle est chauffée.

8. Procédé selon la revendication 7, caractérisé par l'utilisation de modèles perdus produits à partir d'une substance surgelée sous forme de mousse.

9. Procédé selon l'une des revendications précédentes, caractérisé par l'utilisation d'un appareil pour la production de moules de coulée et/ou d'un appareil pour la production de noyaux, l'appareil ou des parties de ce dernier étant contenus dans une chambre de réfrigération.

## Patentansprüche

1. Verfahren zur Herstellung gefrorener Gießformen oder Kerne aus einem körnigen Material und einem Binder in einer Gießkammer oder einem Kernkasten, bei dem ein Binder verwendet wird, der bei positiven Temperaturen, gerechnet in °C, in einem gasförmigen oder flüssigen Zustand ist, dadurch gekennzeichnet, daß der Binder vor dem Mischen mit dem körnigen Material gefroren worden ist.

2. Verfahren nach Anspruch 1, dadurch gekennzeichnet, daß ein Formbinder verwendet wird, der in Form von feinen, dentritischenTeilchen, z.B. Schnee, in dem Formmaterial vorhanden ist, und daß Kompression während des Formvorgangs bewirkt, daß der Binder einen Teil seiner oder seine gesamte Bindekapazität abhängig von den Temperaturbedingungen zur Zeit des Formherstellungsvorgangs erhält.

3. Verfahren nach Anspruch 1, dadurch gekennzeichnet, daß ein Formbinder verwendet wird, der in Form von feinverteiltem pulverisierten Material, z.B. Eis, in dem Formmaterial vorhanden ist, und daß Kompression während des Formvorgangs bewirkt, daß der Binder einen Teil seiner oder seine gesamte Bindekapazität abhängig von den Temperaturbedingungen zur Zeit des Formherstellungsvorgangs erhält.

4. Verfahren nach Anspruch 3, dadurch gekennzeichnet, daß der vorgekühlte Binder in der Form von pulverisiertem Material mit Flüssiggas kombiniert wird.

5. Verfahren nach Anspruch 1, gekennzeichnet durch die Verwendung von Wasserglas und flüssigem Kohlendioxid zur Bildung eines Binders.

6. Verfahren nach Anspruch 1, dadurch gekennzeichnet, daß eine Mischung aus Polyisozyanat und Phenolharz, welches durch Vorgefrieren aktiviert ist, flüssiges Dimethylethylamin oder Triethylamin für die Bildung eines Binders verwendet wird.

7. Verfahren nach einem der Ansprüche 1 bis 6 bei der Herstellung von Gießformen, gekennzeichnet durch die Verwendung von tiefgefrorenen wegzuwerfenden Modellen aus einem Material, das sich beim Erwärmen verflüchtigt.

8. Verfahren nach Anspruch 7, gekennzeichnet durch die Verwendung von wegzuwerfenden Modellen, welche aus einem tiefgefrorenen geschäumten Material hergestellt sind.

9. Verfahren nach einem der vorhergehenden Ansprüche, gekennzeichnet durch die Verwendung einer Vorrichtung für die Herstellung von Gießformen und/oder für die Herstellung von Kernen, wobei die Vorrichtung oder Teile hiervon in einer Kühlkammer enthalten sind.
